



US006461442B1

(12) **United States Patent**  
Bush et al.

(10) **Patent No.:** US 6,461,442 B1  
(45) **Date of Patent:** Oct. 8, 2002

(54) **PROCESS FOR REMOVING A STRIP OF COATING MATERIAL**

(75) Inventors: **Steven D. Bush**, Red Creek, NY (US); **Michael J. Duggan**, Webster, NY (US); **Kathryn A. Wallace**, Canandaigua, NY (US); **Henry T. Mastalski**, Webster, NY (US)

(73) Assignee: **Xerox Corporation**, Stamford, CT (US)

(\*) Notice: Subject to any disclaimer, the term of this patent is extended or adjusted under 35 U.S.C. 154(b) by 0 days.

(21) Appl. No.: **09/450,363**

(22) Filed: **Nov. 29, 1999**

(51) Int. Cl.<sup>7</sup> ..... **B08B 9/04**

(52) U.S. Cl. ..... **134/8**; 134/2; 134/22.1; 134/22.14; 134/22.19; 134/23; 134/25

(58) Field of Search ..... 134/8, 22.1, 22.11, 134/22.14, 22.19, 2, 23, 25, 32

(56) **References Cited**

U.S. PATENT DOCUMENTS

|             |   |         |                 |       |            |
|-------------|---|---------|-----------------|-------|------------|
| 3,862,801 A | * | 1/1975  | Komp            | ..... | 355/15     |
| 3,867,170 A | * | 2/1975  | Ferguson et al. | ..... | 117/37     |
| 4,569,950 A | * | 2/1986  | Hoshi et al.    | ..... | 521/88     |
| 5,352,329 A | * | 10/1994 | Herbert et al.  | ..... | 156/646    |
| 5,378,315 A | * | 1/1995  | Hendrix et al.  | ..... | 156/655    |
| 5,418,349 A |   | 5/1995  | Swain et al.    | ..... | 219/121.84 |

|             |        |              |              |            |       |
|-------------|--------|--------------|--------------|------------|-------|
| 5,424,508 A | 6/1995 | Swain et al. | .....        | 219/121.84 |       |
| 5,628,918 A | 5/1997 | Mastalski    | .....        | 216/8      |       |
| 5,670,291 A | 9/1997 | Ward et al.  | .....        | 430/132    |       |
| 5,893,568 A | 4/1999 | Swain et al. | .....        | 279/2.22   |       |
| 6,001,187 A | *      | 12/1999      | Paley et al. | .....      | 134/6 |

\* cited by examiner

Primary Examiner—Randy Gulakowski

Assistant Examiner—M. Kornakov

(74) Attorney, Agent, or Firm—Robert Thompson

(57)

**ABSTRACT**

A process including providing a hollow imaging drum having a first end, a second end, an outside surface, an inside surface and coating material on both the inside surface and the outside surface at at least the first end, simultaneously contacting the coating material on both the inside surface and the outside surface at the first end of the drum with resilient foam material, flowing liquid solvent for the coating material to the foam material where the foam material contacts the first end of the drum, the foam material being insoluble in the flowing solvent, producing relative movement between the foam material and the drum to simultaneously wipe both the inside surface and the outside surface of the first end of the drum with the foam material and solvent material and simultaneously remove coating material from the inside surface and the outside surface of the first end of the drum, and flowing the solvent away from the drum to carry away coating material removed from the inside surface and the outside surface of the first end of the drum.

**11 Claims, 3 Drawing Sheets**



FIG. 1



FIG. 2



FIG. 3

**FIG. 4****FIG. 5**

**PROCESS FOR REMOVING A STRIP OF  
COATING MATERIAL**

**BACKGROUND OF THE INVENTION**

This invention relates in general to electrostatography and, more specifically, to a system for removing coating material from an end of a drum.

In electrostatography, and particularly in electrophotography, coated substrates such as cylindrical photoreceptor drums (photoreceptors) are commonly used in copier, duplicator, facsimile and multifunctional machines. Photoreceptor embodiments include at least one coating of photosensitive material comprising film forming polymer material, which can be formed on the photoreceptor by known techniques such as immersion or dip coating.

The peripheral ends of a coated photoreceptor are often used to engage members such as spacers, rollers, seals, developer housings, grounding devices and the like. If these members ride on a coated area of the drum, the coating material is rubbed off and the resulting debris can contaminate various components in the machine such as the cleaning system and any optical exposure systems employed in the machine. Also, the coating can interfere with devices that are designed to electrically ground the drum by contacting the outer surface at one end of the drum. Moreover, if the coating thickness is irregular because of poor removal techniques, spacing devices riding on the outside surface of the drum cannot maintain precise spacing between the drum and critical subsystems such as charging, developing, cleaning or other subsystems. Further, if coating material is present in the interior of the drums adjacent the ends of the drum, insertion of supporting end caps may be prevented or hindered. Also, uneven coating deposits in the interior of the drums can cause misalignment of the end caps which, in turn, can cause the drum to wobble during image cycling. The uncoated region at the end of the drum is also necessary to prevent delaminating or cracking of the organic layers at the base of the photoreceptor when the photoreceptor is cycled in an imaging machine. Thus, specified areas at both the outer and inner peripheral ends of a photoreceptor must be free of coating material.

The top of the drum may be maintained free of deposited coating by not immersing a small portion of the upper end of the drum into the coating solution. More specifically, the upper end of the photoreceptor drum can be kept free of coating material by orienting the drum vertically and dipping the drum into a bath of coating material to a predetermined depth which avoids complete immersion of the drum. However, the coating formed over the lower end of the photoreceptor must still be removed or prevented from depositing during dip coating. There are many methods and techniques for accomplishing this. One technique for preventing coatings from depositing is by masking the lower end of the drum prior to dip coating. This technique is time consuming and requires excessive handling. Systems for removing deposited coatings include, for example, laser ablation, mechanically wiping the lower end with blades or brushes and/or by applying solvents to it.

In the laser ablation coating removal technique, a predetermined portion of a coating on a photoreceptor is treated to remove at least part of the coating by directing high energy radiation such as a laser beam and a number of fluid jets at the coating to remove at least part of the coating. This process is often referred to as "laser ablation." The laser ablation process functions to effectively remove at least part of a predetermined portion of a coating without the need for

chemical or mechanical treatments. During laser ablation, the coated substrate is rotated at high speeds. However, a problem is that a rotating cylindrical substrate which is supported only at one end, i.e., a cantilevered state, may sway when the rotation speed is high and/or when the substrate has a relatively small diameter. Swaying of the substrate during for example laser ablation may affect the precision of the ablation process. The laser ablation process is described in detail in U.S. Pat. No. 5,418,349, U.S. Pat. No. 5,424,508 and U.S. Pat. No. 5,628,918, the entire disclosures thereof being incorporated herein by reference. Supplemental devices to reduce drum sway during laser ablation is described in U.S. Pat. No. 5,628,918, the entire disclosure thereof being incorporated herein by reference. 15 Laser ablation systems are complex, expensive and occupy valuable manufacturing space.

Another coating removal method involves using a wiper blade or brush to wipe off the bottom portion of each drum with solvent, to remove the organic polymer films in the intended uncoated region. One technique involves lowering the drum onto a sponge spindle to steady the end of the drum and thereafter, wipe the bottom outside edge of the drum with a flexible wiper blade. This blade wiping system utilizes tapered elastomeric rollers. Each roller is mounted 20 on one end of an arm which has a center pivot point. The other end of the arm carries a wiping blade. As a drum is lowered, the end of the drum engages the tapered end of each roller causing it to offset and move the arm which, in turn, causes the blade to wipe the coating material from the outer 25 surface of one end of the lowered photoreceptor. This method performs well with photoreceptors which require a large coating-free circumferential strip having, for example, a width of 9 millimeters. However, for photoreceptors requiring a relatively small coating-free circumferential strip 30 having, for example, a width of 4 millimeters, consistent, reliable wiping cannot be achieved. Part of this reduction in quality for narrow coating-free circumferential strips is due to the drum wobbling during coating removal, misalignment of the wiper blades on the surface of the drum, and loss of 35 elastomeric roller material as the drum is lowered into contact with the tapered end of the elastomeric rollers. Loss 40 of the material from the rollers causes the rollers to roll erratically rather than smoothly. Moreover, loss of material from the rollers aggravates precise alignment of the drum and blades for cleaning. Also, during lowering, the drum will 45 occasionally contact the blades and dislodge them from alignment. If the rollers are biased against the drum with too much pressure, the drum is pulled off of the mandrel when the mandrel is retracted to remove the drum from the 50 cleaning station. Moreover, the nicked rollers produce debris that deposit on the wiped surface of the bottom of the drum. Replacement and realignment of the rollers requires downtime during which production must be stopped. Further, solvent used to carry away removed coating material often 55 rides up on the rollers and form unwanted coating deposits on the cleaned bottom surface of the drum. Thus, quality control is difficult to maintain. Further, these cleaning systems require frequent replacement of parts, along with attendant downtime. Even with optimization of the bottom 60 edge wipe with wiper blades the reject rate can be as high as 20 to 25 percent.

Another technique for cleaning drums is to utilize brushes with solvents. Because the bristles of the brush tend to flick coating material and solvent during the cleaning operation, the coating material in the imaging area can receive unwanted solvent and/or coating material from the brushes during the cleaning operation. These cleaning devices

become less efficient and reliable when the cleaned strip at the end of the drum has a very small width, for example, about 4 mm wide.

Thus, each coating prevention or removal technique has its advantages and disadvantages. In all cases, there should be little or no residual organic polymer in the bottom uncoated area or it is considered defective for the reasons described above. To prevent defective photoreceptors from getting to the customers, it is necessary to carefully inspect each photoreceptor to detect these defects during the manufacturing process. Therefore, a very large amount of time and expense is required to weed out otherwise acceptable photoreceptors.

#### INFORMATION DISCLOSURE STATEMENT

U.S. Pat. No. 5,418,349 issued to Swain et al on May 23, 1995—A process is disclosed for treating a coated substrate to reduce the thickness of the coating involves directing a laser beam at a predetermined surface portion of the substrate to remove part of the coating. The process can be used to treat a coated photoreceptor to precisely reduce the thickness of the coating in a predetermined region.

U.S. Pat. No. 5,424,508 issued to Swain et al on Jun. 13, 1995—A system is disclosed for removing a band of coating material from a first end of a coated cylinder having a second opposite end including ablating the band of coating material with a laser beam and directing an annular curtain of compressed fluid against the band in a direction away from the second opposite end to create an air curtain along the outer surface of the cylinder in a direction from the second opposite end toward the band and the first end.

U.S. Pat. No. 5,628,918 issued to Mastalski on May 13, 1997—A method is disclosed comprising: (a) rotating a hollow cylindrical substrate having a coating thereon; (b) employing a gas bearing around the circumference of the rotating substrate along a portion of the length of the substrate to provide support to the substrate during its rotation; and (c) removing a portion of the coating.

U.S. Pat. No. 5,670,291 issued to Ward et al on Sep. 23, 1997—A process is disclosed for fabricating an electrophotographic imaging member including providing a substrate coated with at least one photoconductive layer, applying a coating composition to the photoconductive layer by dip coating to form a wet layer, the coating composition comprising finely divided amorphous silica particles, a dihydroxy amine charge transport material, an aryl charge transport material that is different from the dihydroxy amine charge transport material, a crosslinkable polyamide containing methoxy groups attached to amide nitrogen atoms and a crosslinking catalyst, at least one solvent for the hydroxy amine charge transport material, aryl charge transport material that is different from the dihydroxy amine charge transport material and the crosslinkable polyamide, and heating the wet layer to crosslink the polyamide and remove the solvent to form a dry layer in which the dihydroxy amine charge transport material and the aryl charge transport material are molecularly dispersed in a crosslinked polyamide matrix.

U.S. Pat. No. 5,893,568 issued to Swain et al on Apr. 13, 1999—A device is disclosed for supporting a hollow substrate having two open ends in an aligned orientation, wherein one end of the substrate is engageable with a chuck assembly, including: (a) a base for contacting the other end of the substrate; (b) a post coupled to the base, wherein a section of the post is positioned within the substrate, thereby defining a substrate disposed post section; and (c) a spring

apparatus coupled to the substrate disposed post section, wherein the spring apparatus is disposed within the substrate and contacts the substrate interior surface, wherein the spring apparatus is compressed by the substrate during misalignment of the substrate with the device and the compressed spring apparatus springs back to push the substrate to the aligned orientation with the device.

#### BRIEF SUMMARY OF THE INVENTION

It is, therefore, an object of the present invention to provide an improved edge cleaning system for electrostatographic imaging drums.

It is another object of the present invention to provide an improved edge cleaning system for electrostatographic imaging drums.

It is still another object of the present invention to provide an improved edge cleaning system for electrostatographic imaging drums that reliably removes circumferential strips of coating material having a narrow width as well as those having a wide width.

It is yet another object of the present invention to provide an improved edge cleaning system for electrostatographic imaging drums having excellent wiping capabilities.

It is another object of the present invention to provide an improved edge cleaning system for electrostatographic imaging drums which forms high quality cleaned circumferential strips.

It is still another object of the present invention to provide an improved edge cleaning system for electrostatographic imaging drums that is easier to maintain and reduces maintenance.

It is yet another object of the present invention to provide an improved edge cleaning system for electrostatographic imaging drums which is less complex.

It is another object of the present invention to provide an improved edge cleaning system for electrostatographic imaging drums which avoids damage during cleaning cycles.

It is still another object of the present invention to provide an improved edge cleaning system for electrostatographic imaging drums which simultaneously wipes both the inside and outside of the bottom edge of a coated photoreceptor.

It is yet another object of the present invention to provide an improved edge cleaning system for electrostatographic imaging drums which is easier to set up and maintain.

The foregoing objects and others are accomplished in accordance with this invention by providing a process comprising

providing a hollow imaging drum having  
a first end, a second end,  
an outside surface,  
an inside surface and  
coating material on both the inside surface and the  
outside surface at at least the first end,  
simultaneously contacting the coating material on both  
the inside surface and the outside surface at the first end  
of the drum with resilient foam material,  
flowing liquid solvent for the coating material to the foam  
material where the foam material contacts the first end  
of the drum, the foam material being insoluble in the  
flowing solvent,  
producing relative movement between the foam material  
and the drum to  
simultaneously wipe both the inside surface and the  
outside surface of the first end of the drum with the  
foam material and solvent material and

simultaneously remove coating material from the inside surface and the outside surface of the first end of the drum, and

flowing the solvent away from the drum to carry away coating material removed from the inside surface and the outside surface of the first end of the drum.

#### DESCRIPTION OF THE DRAWINGS

A more complete understanding of the present invention can be obtained by reference to the accompanying drawings wherein:

FIG. 1 is a schematic front view in elevation of a cleaning assembly of this invention.

FIG. 2 is a schematic plan view of the cleaning assembly shown in FIG. 1.

FIG. 3 is a schematic side view in elevation of a cleaning assembly of this invention.

FIG. 4 is a schematic plan view of the cleaning foam of this invention.

FIG. 5 is a schematic illustration in elevation of the foam shown in FIG. 4.

These figures merely schematically illustrate the invention and are not intended to indicate relative size and dimensions of the device or components thereof.

#### DETAILED DESCRIPTION OF THE DRAWING

For purposes of illustration, the process according to the invention will be described with reference to the treatment of a coated cylindrical photoreceptor.

Referring to FIGS. 1, 2 and 3, a cleaning assembly 10 of this invention is shown comprising a cleaning foam 12 retained in a housing 14 comprising a bowl ring 16 removably mounted on a base 18. Secured to base 18 is at least one threaded spike 20 which penetrates cleaning foam 12 and prevents it from turning during cleaning. An optional bowl lip 22 along the upper periphery of bowl ring 16 ensures retention of cleaning foam 12 during cleaning. Any suitable housing 14 may be utilized to retain the cleaning foam 12 during the coating removal operation. The housing may be solid, foraminous, notched, and the like. The housing should be sufficiently rigid to retain the foam in position during the cleaning operation. Generally, where a bowl lip 22 is omitted, the cleaning foam 12 is sufficiently compressed when confined within the housing 14 to achieve a friction fit which retains the foam in the housing during the coating removal cycle. Alternatively, retaining members may be used to prevent slippage. Any suitable retaining member may be utilized. Typical retaining members include, for example, pins, spikes, knurled interior surfaces of the housing (not shown) and the like. Secured to and extending upwardly from base 18 is a hollow shaft 24 having an upper externally threaded end. Coaxially enclosed within and spaced from hollow shaft 24 is a vent tube 26. A resilient guide spindle 28 is positioned around shaft 24 and on top of cleaning foam 12.

Cleaning foam 12 contains a circular slit 29 having a diameter equal to or slightly smaller than the largest diameter of resilient guide spindle 28. Pin washer 30 carries at least one pin 32 which becomes imbedded into resilient guide spindle 28 when threaded screw cap 34 is screwed onto the upper threaded end of hollow shaft 24. Threaded screw cap 34 also presses resilient guide spindle 28 against cleaning foam 12 to ensure retention of cleaning foam 12 within housing 14 during the cleaning operation. Base 18 is securely fastened to shaft flange 36 by a plurality of bolts 38.

Spacer ring 40 is sandwiched between base 18 and shaft flange 36 with O-rings 42 and 44 providing solvent tight seals to allow solvent to be fed through hollow connecting passageways extending through shaft flange 36, spacer ring 40, base 18, hollow shaft 24 and screw cap 34. Screw cap 34 contains at least one exit opening 46 to allow solvent to exit screw cap 34 and flow downwardly over guide foam 28 onto cleaning foam 12. Guide spindle 28 contains at least one groove 48 to enhance flow of solvent to clean cleaning foam 12. Instead of, or in combination with, flow of solvent from exit opening 46, solvent may be fed directly to cleaning foam 12 by holes or ducts (not shown) in hollow shaft 24 or base 18 adjacent to cleaning foam 12. Shaft flange 36 also carries a ball plunger 50 and a quarter turn pin slot 52. Hex nut 54 facilitates adjustment of ball plunger 50.

Also shown in FIG. 3 is a drive shaft 56 driven by a drive device 58. Drive shaft 56 has a pin 59 which aids in connecting shaft 56 to flange 36. Any suitable drive device 58 may be utilized. Typical drive devices include, for example, a gear box, a smart motor, an air driven motor, and the like. When activated, drive device 58 causes cleaning assembly 10 to rotate around an imaginary axis or centerline. A coated drum 60 carried by reciprocatable chuck 62 is advanced downwardly over resilient guide spindle 28 and into circular slit 29 for simultaneous removal of coating material from a circumferential strip on the inside surface and outside surface of the lower end of drum 60. Upon completion of coating removal, reciprocatable chuck 62 is retracted to remove drum 60 from cleaning assembly 10.

Illustrated in FIGS. 4 and 5 is a cleaning foam 12 of this invention. Cleaning foam 12 contains a circular slit 29 which extends vertically downwardly from the substantially horizontal upper surface 70 of cleaning foam 12. A centered, axially aligned hole 72 allows foam 28 to be slid down on hollow shaft 24 against base 18 (see FIGS. 1 and 3). Circular slit 29 is connected by at least one shallow drain groove 76 which radiates from circular slit 29 to the outer circular wall 78 of cleaning foam 12. Circular wall 78 is perpendicular to the upper surface 70. Shallow drain groove 76 channels solvent and dissolved coating material from circular slit 29 toward the outer periphery of circular wall 78 of cleaning foam 12 during removal of coating material from one end of coated drum 60 (see FIG. 3). The drain grooves 76 or any other suitable channel or channels prevents the formation of puddles which can cause a meniscus leading to wicking of the solvent and dissolved coating material to the outer layer of the photoreceptor which in turn causes an undesirable uneven wipe height.

In operation and referring to FIG. 3, a coated hollow imaging drum 60 having a first lower end, a second upper end, an outside surface, an inside surface and coating material on both the inside surface and the outside surface at the first lower end, is lowered downwardly by reciprocatable chuck 62 by conventional drum transport devices (not shown) over the tapered upper end of guide foam 28 which aids in centering drum 60. Drum 60 is mounted on chuck 62 such that its longitudinal axis is vertically oriented. Although a preferred vertical orientation of the drum 60 and cleaning assembly 10 is illustrated, any other suitable orientation may be utilized instead. Typical non-vertical orientations include, for example, horizontal and diagonal orientations. Drum 60 is preferably mounted using a conventional chucking device 62 coupled to a drum transport mechanism (not shown). Drum transport mechanisms are well known and described for example, in U.S. Pat. No. 5,334,246, the entire disclosure thereof being incorporated herein by reference. The transport mechanism (not shown)

may move coated drum 60 to and from the coating removal station. Any suitable conventional chucking device may be utilized. A typical chuck comprises a shaft and inflatable rubber air bladder disclosed, for example, in U.S. Pat. No. 4,783,108, the entire disclosure thereof being incorporated by reference. Lowering of drum 60 is continued until the lower end of drum 60 slides into circular slit 29 of cleaning foam 12 to a predetermined depth. The predetermined depth ensures that the adjacent vertical walls of slit 29 contact the region of the end of drum 60 from which coating material is to be removed by the cleaning foam 12. Thus, the adjacent vertical walls of slit 29 simultaneously contact the coating material on both the inside surface and the outside surface at the first lower end of the drum with cleaning foam 12. Therefore, to remove a circumferential strip of the coating from the bottom of coated drum 60 as cleaning assembly 10 rotates, drum 60 is lowered toward cleaning foam 12 and the bottom edge of drum 60 is slid into slit 29 to a predetermined depth corresponding to the width of the strip of coating material to be removed. Alternately, drum 60 need not be lowered and, instead, the cleaning assembly 10 may be raised (not shown) to a height where the bottom end of drum 60 slides into slit 29 in foam 12. Drum 60 may be rotated (not shown) or the foam 12 may be rotated, or both drum 60 and foam 12 may be rotated (not shown) to achieve relative movement between the foam and the drum surface during coating removal.

Liquid solvent is pumped from any suitable source by conventional pumps such as gear pumps, centrifugal pumps, and the like (not shown) through passageways in drive shaft 56, the passageways in cleaning assembly 10 and out exit openings 46 and/or through other suitable openings in hollow shaft 24 or flange 36 (not shown) adjacent foam 12. The solvent flows down the outer surface of guide foam 28, including along grooves 48, into slit 29, under the lower end of the drum, up out of slit 29 and along drain grooves 76. Preferably a limited amount of the solvent also flows over much of the upper surface 70 of cleaning foam 12 not occupied by the shallow drain groove 76 to remove coating material residue and prevent carry over of this residue to the next drum to be cleaned.

As the solvent flows from the inside surface of drum 60 to the outside surface of the lower end of drum 60, it coats those surfaces of foam 12 in slit 29 which contact the interior and exterior regions of the end of drum 60 from which coating material is to be removed. It is preferred that the solvent flow to the contacting interface between the inside surface of drum 60 and the adjacent foam 12, then under the bottom of drum 60 to the contacting interface between the outside surface of drum 60 and the adjacent foam 12, and then along the exposed upper surface 70 of the foam 12, including the channels 76, the solvent and dissolved coating material finally overflowing from housing 14 down into any suitable device, such as a catch tray (not shown). The supplying of a fluid flow of solvent to the contacting interfaces between the inside surface of drum 60 and the adjacent foam 12 and contacting interface between the outside surface of drum 60 and the adjacent foam 12 during the coating removal treatment prevents debris from building up at the drum end during the coating removal process. Thus, the solvent flows from the contacting interfaces between the inside surface of drum 60 and the adjacent foam 12 and contacting interface between the outside surface of drum 60 and the adjacent foam 12 toward the outer periphery of foam 12. This prevents coating buildup on the foam, prevents redeposit of the coating material onto the drum and increases the online production time of the cleaning system.

The solvent flow rate depends upon a number of variables including drum size, the width of the strip of coating material to be removed, the thickness of the coating material, the specific coating material to be removed, the specific solvent and the like. Preferably, the fluid flow should be sufficient to carry away the highly concentrated solution of coating material dissolved in solvent and prevent redeposit of the coating material back onto the drum surface. Generally, the size and number of drain grooves or other suitable channels in the cleaning foam along with the amount of solvent being fed to the slit should be chosen to allow the solvent to escape without any splashing occurring during the removal of the drum from the foam slit after cleaning is completed. For example, any build up of solvent within the interior of the drum during cleaning should be avoided because the solvent will rush out of the interior of the drum and splash up onto the unwiped area of the drum causing a defect when the drum is removed from the slit. As foam 12 rotates during the cleaning process, a circumferential strip of coating material is removed from the bottom end of drum 60, exposing the underlying insoluble cylindrical photoreceptor substrate. The foam 12 remains in contact with the predetermined portion of the end of drum 60 until the intended amount of coating has been removed. The duration for wiping varies with the amount of pressure exerted against the drum, the total contact area and the like. When the desired amount of coating has been removed from the outer predetermined surface of drum 60, the drum and foam 12 are separated. Once the inner and outer predetermined portions of drum 60 have been treated, the coating removal process is stopped and drum 60 may move on to another processing station or removed from the chucking device for further processing or use.

In the embodiment shown in FIG. 3, the cleaning assembly is rotated about its axis by drive device 58 to achieve relative movement and scrubbing contact between the surfaces of foam 12 in slit 29 and the adjacent interior and exterior surfaces of drum 60. Alternatively, the cleaning assembly may be stationary and the chuck and drum may be rotated or both the cleaning assembly and the chuck and drum may be rotated in opposite directions to achieve relative motion between the contacting foam material and the drum surface. This relative movement between the foam material and the drum simultaneously removes coating material from the inside surface and the outside surface of the lower end of the drum. Generally, it is preferred that the foam 12 is not vertically reciprocated, but merely rotated with the drum being lowered down into the circular slit 29.

The cleaning assembly 10 is preferably rotated about its longitudinal axis during the removal of the coating. The speed of rotation varies with the diameter of the drum, the width of the circumferential region to be cleaned, the thickness of the coating or coatings, the materials of the coatings, the solvent, the temperature, the foam material, the contact pressure between the foam material and drum, and the like. A typical cleaning foam housing rotational speed rpm is about 35 rpm. However, speeds greater or less than 35 rpm may be utilized so long as the cleaning objectives of this invention are satisfied. Excessive speed reduces wiping quality and the solvent begins to function as lubricant with less shear and friction, thereby reducing the wiping effectiveness because the foam merely rides (surfs) on top of the solvent without adequately contacting the coating and drum substrate.

The substrate for coated drum 60 may comprise any suitable material. Typical materials include, for example, aluminum, nickel, zinc, chromium, stainless steel, cadmium,

titanium, metal oxides, plastics, composites, and the like. The substrate may comprise one layer or a plurality of layers, for example conductive layer coated over an insulating layer. The thickness of the substrate can vary widely depending on the intended use of the photoreceptor, and preferably is from about 65 micrometers to about 5 millimeters thick, most preferably from about 0.05 millimeter to about 2 millimeters thick. However, thicknesses outside these ranges may be utilized where suitable. The substrate is insoluble in the solvents employed for coating removal. There does not appear to be any criticality as to the diameter of the drum, thickness of the drum, length of the drum, or the material of the drum.

The process of this invention removes various types of known photoreceptor coatings which can be dissolved with a solvent. These coating can include one more layers, and typically will include multiple layers such as a blocking layer, a charge generating (photogenerating) layer, a charge transporting layer and an optional overcoat layer. Thus, preferably, all of the solvent soluble coating layers present at the outer and inner peripheral end region of the photoreceptor are removed.

The coating removed preferably includes, as a photoconductive material, one or a plurality of layers of organic resins carrying dispersed photoconductive materials. Such coatings include, for example, a photoconductive material such as pigments dibromoanthrone, metal-free and metal phthalocyanines, halogenated metal phthalocyanines, perylenes, azo pigments, and the like carried in a suitable organic binder resin. Examples of typical organic binder resins include polycarbonates, acrylate polymers, vinyl polymers, cellulose polymers, polysiloxanes, polyamides, polyurethanes, polyesters, block, random or alternating copolymers thereof, and the like.

The layer or layers of coatings on the drums are formed using well-known techniques and materials. For example, the coatings may be applied to the drum substrate by immersion, spray coating, dip coating, or the like. Dip coating or spray coating is preferred. Typical coating techniques and materials are illustrated in U.S. Pat. No. 5,091,278, U.S. Pat. No. 5,167,987 and U.S. Pat. No. 5,120,628, the entire disclosures thereof being incorporated herein by reference. The process of this invention can be carried out in conjunction with a coating process, preferably after the coating has partially hardened. Although removal of a partially dried coating is preferred, removal of dried coatings may also be accomplished with the process of this invention.

Any suitable solvent may be employed with the foam 12 to remove the coating material from the bottom of drum 60. Typical solvents include, for example, methylene dichloride, tetrahydrofuran, toluene, n-butyl acetate, n-butyl alcohol, xylene, and the like.

Any suitable resilient solvent resistant foam material may be utilized for cleaning foam 12. Preferably, the foam material comprises cellular synthetic solvent resistant polymer material generally resembling natural sponge. Typical solvent resistant foam materials include, for example, polyethylene, polypropylene, neoprene, and the like which do not dissolve or swell in the solvent employed for coating removal. Selection of the solvent resistant foam depends upon the specific cleaning solvent utilized. Thus, for example, neoprene is solvent resistant to xylene, n-butyl alcohol and n-butyl acetate, but is not resistant to tetrahydrofuran.

The foam pores may be closed cell or open cell. Most of the cells along the outer surface and in the walls of circular

slit 29 of the foam 12 are open cells for more uniform removal of solvent and dissolved coating material and migration of removed dissolved coating material. These open cells are present even with closed cell foam because the cutting operation to fabricate and shape the foam, cuts open the closed cells along the surfaces cut. Generally, an average cell diameter of between about 1 millimeter and about 3 millimeters is preferred. Also preferred is a cell size having an average diameter less than about the width of the area at the bottom of the drum which is to be cleaned. However, cell sizes outside these ranges may be employed so long as the cleaning objectives of this invention are satisfied. The cell walls of the foam should be sufficiently stiff to provide a scrubbing action which, with the aid of liquid solvent removes the coating material from the bottom of the drum. A >6 lb. foam material of closed cell polyethylene provides optimum results. However, foam material greater than or less than about >6 lb. may be employed so long as the cleaning objectives of this invention are satisfied. The foam material should be solvent insoluble and sufficiently resilient to rapidly return to its original shape after being deformed by pressure.

The circular slit 29 is concentric with the imaginary rotational axis of cleaning assembly 10. The diameter of the circular slit, when the foam is in the free uncompressed state, is preferably about same as the outside diameter of the drum being treated. Some foams exhibit a limited amount of expansion which can be controlled by the bowl ring. Generally, at least some compression of the sponge is desirable to exert sufficient pressure against the interior and exterior surfaces of the drum during cleaning.

When the foam in the housing is viewed with the naked eye from above (plan view) prior to insertion of the drum into the slit, the slit is substantially invisible or barely discernable because the opposing sides of the slit are in contact with each other. Generally, the slit in the foam for receiving the end of the drum is preferably cut substantially vertically into the foam. However, limited deviation from vertical may be tolerated, particularly where the width of the area to be cleaned is narrow. Thus, preferably, the opposing walls on each side of the slit are vertical and substantially parallel with the outer and inner contacting surfaces of the drum. The depth of the slit does not appear to be critical, and may extend all the way to the bottom of the cleaning foam. Also, depending on the width of the strip to be cleaned of coating material, the degree (distance) of drum insertion into the slit may vary for different production runs of different photoreceptors. Thus, the amount of interference contact due to entry of the drum into the foam slit can vary for different production runs, even though the same foam is used for coating removal. Typical widths of cleaned bottom edges of drums extend from about 0.5 millimeter to about 15 millimeters. Preferably, the cleaning foam is utilized to remove a coating in a strip having a width between about 3.5 millimeters and about 9 millimeters. Generally, if the strip of coating material on the drum is too wide, too much coating material must be carried away by the solvent and solvent flow, and complete cleaning may be difficult to achieve.

The cleaning foam 12 may comprise one or more separate sections. A one-piece foam is preferred for convenience in fabrication, installation, and replacement. Also, a one-piece foam is less likely to become dislodged during use, particularly at the point in time when the drum is separated from the cleaning foam after cleaning. Multiple section foams can be of any suitable shape. For example, a disk shaped section (corresponding to the inner section circumscribed by the circular slit 29) can be used for the central section of the

## 11

foam and the outer section can be donut shaped with the disk shaped section filling the hole in the donut shaped section. Thus, the expression "cleaning foam", as employed herein is defined as a foam comprising one or more sections.

Preferably, the top of the foam is flat for more precise cleaning within the predetermined boundaries of the region to be cleaned. The outer sides extending from the top to the bottom of the foam may be of any suitable shape such as vertical or inclined. The outer plan view shape of the foam may be of any suitable configuration. Typical configurations include circular, square, octagonal, oval, and the like. However, a circular shape, when viewed in elevation, is preferred for simplicity in installation and minimization of space occupied.

Generally, the foam is slightly larger than the housing in which it is confined. Thus, it is slightly compressed after installation in the housing and is retained therein by a friction fit. This friction fit also ensures that the walls of the slit in the foam exert sufficient pressure against the adjacent surfaces of the drum during removal of a strip of coating material from an end of the coated drum. Therefore, the foam in the housing should exert sufficient pressure to remove the desired amount of the particular coating to be treated. The overall dimensions of the foam change very little due to the slight compression imposed when installed in a housing. The height of the foam does not appear to change after installation in the housing.

The cleaning foam may be fabricated by any suitable means. For example, for a foam 12 having round plan view configuration, the foam may be cut with a hole saw. Drain grooves 76 to allow the solvent and dissolved coating material to drain away may be fabricated by, for example, a "U" shaped razor blade. Any other suitable fabrication device may be utilized such as a carbon dioxide laser, air knife (using high pressure and a small tip), water knife, and the like. If desired, internal channels (not shown) extending radially from the circular slit to the outer periphery of the cleaning foam may be utilized in place of or in addition to the external drain grooves. Such internal channels may be formed by any suitable technique such as drilling, hot wire, cutting, stamping, molding and the like.

The flow rate of the solvent carrying dissolved coating material away from the end of the drum can be increased by any suitable technique including, for example, increasing the number and size of external and/or internal drain channels. Increasing the rpm of the cleaning assembly can also increase solvent removal flow, but an increase in rpm tends to decrease the quality of coating removal as described above.

The process of this invention provide an improved edge cleaning system for electrostatographic imaging drums that reliably removes circumferential strips of coating material having a narrow width as well as those having a wide width. The edge cleaning system of this invention is also easier to maintain, reduces maintenance and is less complex. Further, the edge cleaning system of this invention avoids damage to cleanings system components during cleaning cycles. Also, the edge cleaning system of this invention simultaneously wipes both the inside and outside of the bottom edge of a coated photoreceptor. Moreover, the process of this invention greatly facilitates set up of the cleaning system and eases replacement of a cleaning head in the cleaning foam equipped systems.

#### PREFERRED EMBODIMENT OF THE INVENTION

A number of examples are set forth hereinbelow and are illustrative of different compositions and conditions that can

## 12

be utilized in practicing the invention. All proportions are by weight unless otherwise indicated. It will be apparent, however, that the invention can be practiced with many types of compositions and can have many different uses in accordance with the disclosure above and as pointed out hereinafter.

#### EXAMPLE I

Hollow aluminum drums were provided. Each of these 10 drums were dip coated to form a charge generator layer coating comprising organic photoconductive particles dispersed in a thermoplastic polymer binder and a charge transport layer comprising small molecule charge transport molecule dissolved in a polycarbonate thermoplastic polymer binder. Because these drums were dip coated, the charge 15 generator and charge transport coatings extended to the very edge of at least one end of each of the drums.

#### EXAMPLE II

Drums described in Example I were bottom edge wiped to 20 remove a 3.5 millimeter width of the coatings from the coated end of each drum. Bottom edge wiping was effected by using a machined disk shaped closed cell >6 lb. polyethylene cleaning foam having an outside diameter of 50 25 millimeters and a height of 19 millimeters. The average pore size of the foam was between 1 and 3 millimeters. The foam had a 10 millimeter diameter hole along its axis and four evenly spaced notches along its upper periphery similar in 30 configuration to that illustrated in FIGS. 4 and 5. Concentric with the hole along the axis was a slit extending from the top of the foam to a depth of 12 millimeters. Each of the notches had a depth of 5 millimeters and a width of 10 millimeters at the slit flaring to a width of 14 millimeters at the outer 35 edge of the foam disk. This foam disk was mounted in a snugly fitting bowl shaped holder of a cleaning assembly similar to that illustrated in FIGS. 1-3 by sliding the foam down over a resilient guide spindle having a diameter equal to the 39 millimeter inside diameter of the coated drum. The 40 cleaning foam was prevented from turning relative to the bowl shaped holder by four spikes extending upwardly from the holder through the foam. The drum was lowered into the slit for a distance of 3.5 millimeters and the cleaning assembly was rotated 35 rpm. Tetrahydrofuran solvent for the 45 thermoplastic polymer binders in the charge generator layer coating and the charge transport layer coating was fed to the top of the guide spindle and allowed to flow down the sides of the spindle, into the slit, out of the slit and away from the drum in the notches and along the top of the foam disk. After the coatings at the end of the lower end of the 50 drum were removed by the rotating cleaning assembly, the drum was raised away from the cleaning assembly. Examination of the wiped bottom edge of the drums revealed excellent removal of the coating with an even edge between the cleaned area and the remaining coated area.

#### EXAMPLE III

The process described in Example II was repeated with 55 other foam materials including urethane foam, natural latex foam and neoprene foam substituted for the polyethylene cleaning foam. Examination of the wiped bottom edge of the drums revealed defects due to deposits of particles of foam resulting from disintegration of the cleaning foams during cleaning.

Although the invention has been described with reference to specific preferred embodiments, it is not intended to be limited thereto, rather those having ordinary skill in the art

## 13

will recognize that variations and modifications may be made therein which are within the spirit of the invention and within the scope of the claims.

What is claimed is:

1. A process comprising for removing a coating material providing a hollow imaging drum having
  - a first end, a second end,
  - an outside surface,
  - an inside surface and
  - coating material on both the inside surface and the outside surface at at least the first end,
 simultaneously contacting the coating material on both the inside surface and the outside surface at the first end of the drum with resilient foam material,
  - flowing liquid solvent for the coating material to the foam material where the foam material contacts the first end of the drum, the foam material being insoluble in the flowing solvent,
  - producing relative movement between the foam material and the drum to
  - simultaneously wipe both the inside surface and the outside surface of the first end of the drum with the foam material and solvent material and
  - simultaneously remove coating material from the inside surface and the outside surface of the first end of the drum, and
  - flowing the solvent away from the drum to carry away coating material removed from the inside surface and the outside surface of the first end of the drum.
2. A process according to claim 1 wherein the foam material comprises a foam having a substantially horizontal upper surface and a vertical circular slit in the upper surface to receive the first end of the drum for simultaneous wiping

## 14

of both the inside surface and the outside surface of the first end of the drum with the foam material.

3. A process according to claim 1 wherein the foam material comprises a foam having a substantially horizontal upper surface.

4. A process according to claim 3 wherein the foam material has a disk shape with a circular wall which is perpendicular to the substantially horizontal upper surface and coaxial with a vertical circular slit.

5. A process according to claim 4 wherein the substantially horizontal upper surface has at least one drain groove extending radially from the slit to the circular wall to channel flowing solvent and coating material away from the drum.

6. A process according to claim 4 including rotating the foam material while maintaining the drum stationary to produce relative movement between the foam material and the drum.

7. A process according to claim 1 wherein the foam material comprises closed cell foam.

8. A process according to claim 1 wherein the foam material comprises polyethylene.

9. A process according to claim 1 wherein the foam material comprise cells having an average cell diameter of between about 1 millimeter and about 3 millimeters.

10. A process according to claim 1 including removing a strip of coating material from the outside surface of the first end of the drum, the strip having a width between about 3.5 millimeters and about 9 millimeters.

11. A process according to claim 1 wherein the foam material is compressed against the drum while simultaneously wiping both the inside surface and the outside surface of the first end of the drum.

\* \* \* \* \*